# EUROPEAN PATENT APPLICATION

(11) **EP 3 859 034 A1**
(43) Date of publication of application: **04.08.2021**
(21) Application number: 21460002.5
(22) Date of filing: 07.01.2021
(51) Int. Cl.: C22C 38/00, C22C 38/02, C22C 38/10, C22C 1/02, C22C 45/02, H01F 1/153, C21D 8/12, C22C 33/00, C21D 1/84

(54) **BULK NANOCRYSTALLINE IRON ALLOY**

(30) Priority: 28.01.2020 PL 43272820
(71) Applicant: Politechnika Czestochowska, 42-201 Czestochowa (PL)
(72) Inventor: Nabialek, Marcin, 42-200 Czestochowa (PL); Bloch, Katarzyna, 42-231 Cykarzew Pólnocny (PL); Jez, Bartlomiej, 97-510 Reczno (PL)

(57) **Abstract**

Nanocrystalline bulk iron alloy, characterised in that it has the atomic composition Fe₆₅Co₁₁₋ₓB₂₀SiₓZr₂Hf₂, where the value of x is equal to: 0.25 or 0.5 or 0.75 or 1, and in which the permissible quantity of impurities does not exceed 0.09 %.

## Description

The subject of this invention is a bulk nanocrystalline alloy based on iron, and classified as a soft magnetic alloy, which could find applications in electronic, electrical, industrial and power branches of engineering; particularly in components for: high power transformers for impulse/drive power systems, high accuracy current transformers for energy meters or pulse transformers for communication systems.

In modern technology, soft magnetic materials have been used widely and their range has been expanded thanks to the development of, amongst others, nanocrystalline alloys. In the conversion of electricity, a very important role is played by inductors, essential components of which are cores made of magnetically soft materials. In addition to conventional materials, modern materials are used increasingly, i.e.: amorphous alloys and nanocrystalline alloys. The structure of nanocrystalline alloys is two-phase: equiaxed crystals with an average size not exceeding 20 nm are distributed evenly within an amorphous matrix.

The content share of the crystalline phase is approximately 60-70 % by volume. The soft magnetic behaviour of these materials is related to the ultra-fine-grained structure and the random crystallographic orientation of the grains in space. There is a limit on the grain size, above which the coercive field grows radically, and this limiting size amounts to approximately 40-60 nm, depending on the composition of the alloy.

This is a clear limit, below which we can speak of a nanocrystalline material, defined by a radical change in the material properties; and not, as is often assumed, an arbitrary value, e.g. 100 nm - not related to a qualitative change in structure or properties. The technology of soft magnetic alloys of iron and cobalt comprises of two-stages: the first stage is the casting of an amorphous alloy in the form of a strip, and in the second stage, partial crystallisation of the alloy takes place, due to appropriate heat treatment. Currently, three basic types of nanocrystalline alloys are known: FINEMET (Fe-Nb-Cu-Si-B), NANOPERM (Fe-Zr-Cu-B) and HITPERM (Fe-Co-Zr-Cu-B).

The first two groups of alloys can be used at temperatures not exceeding 230 °C, while the alloys of the third group retain good magnetic properties at temperatures of up to 550 °C.

The high rate of cooling from the liquid state - necessary to obtain an amorphous structure - forces these special alloys to form; the vast majority of these alloys are tapes with a thickness not exceeding 40 µm. The functional properties of nanocrystalline alloys are determined by their composition and structure, i.e. these properties depend on the chemical composition and heat treatment.

Various compounds and alloys with properties such as saturation magnetisation, Curie temperature and coercive field value are known from industrial practice. For example, as a result of the development of a stable and reliable production process for nanocrystalline materials, with negligible magnetostriction effect, one of the most perfect nanocrystalline composite materials, Fe73.5Cu1Nb3Si15.5B7, was obtained; this formula represents the class of soft magnetic materials known by the trade name of Vitroperm. This material has a two-phase structure, consisting of ultra-fine silica grains, each with a diameter of 10-20 nm, deposited during the final stage of production of the amorphous phase. As a result, the magnetocrystalline anisotropy (this is how the structure of the material is described in the literature) disappears through averaging, as does the saturation of magnetostriction. Consequently, these materials can achieve the highest permeability with the lowest coercivity. This material is produced in large quantities by Vacuumschmelze.

Polish Patent No. 154378 describes an amorphous metal alloy, magnetically soft, intended in particular for magnetic cores operating in variable magnetic fields of increased frequency and impulse fields, being on the Fe matrix and containing 18 - 21 % by weight Co, 4 - 8 % B and Si in total and 0.05 - 1.0 % Ta, with the balance of the composition being Fe. Another material, known from Polish Patent No. 131127, is a metal alloy of iron, boron and silicon, containing by weight: (77 ÷ 80 %) iron, (12 ÷ 16 %) silicon, (5 ÷ 10 %) boron and traces of impurities; this material is produced in the form of thin tapes.

The aim of the currently described invention is to obtain a massive nanocrystalline, rapidly-cooled iron alloy, the properties of which will be characterised by a low value of coercive field, high saturation induction and excellent temperature stability. The alloy itself is obtainable in a single-step process.

The subject of the invention is a nanocrystalline iron alloy, characterised by its composition of Fe₆₅Co₁₁₋ₓB₂₀SiₓZr₂Hf₂, where x is: 0.25 or 0.5 or 0.75 or 1. The balance of the material comprises of unavoidable impurities; such unavoidable contamination amounts to a maximum of 0.09 %.

According to the invention, the bulk, rapidly-cooled nanocrystalline alloy, the main component of which is iron, is characterised in that Si (Si: 0.25 or 0.5 or 0.75 or 1 %) is introduced as a structural stabiliser. Increasing the Si content blocks the growth of the Fe phase and borides by limiting the diffusion of atoms over longer distances.

The massive nanocrystalline alloy was produced in a single production stage, which means that it was not subjected to additional treatment. To enable its nanocrystallisation in the casting process, it was cooled at a rate of approximately 102 K/s; such a speed causes significant relaxation of the structure and gives the alloy the expected properties. According to the invention, the material of the Fe₆₅Co₁₁₋ₓB₂₀SiₓZr₂Hf₂ alloy contains (atomically): Fe - 65 %; B - 20 %; Zr - 2 %; Si - from 0.25 % to 1 %; Co - from 10 % to 10.75 %, Hf - 2 % when the Coll-xSix relationship is satisfied (where: x = 0.25 or 0.5 or 0.75 or 1) with the permissible contamination of not greater than 0.09 %.

According to the invention, the advantage of the proposed alloy is also that, in relation to amorphous materials, produced in the form of thin strips of alloy, they can be produced in one production step with a thickness of 0.5 mm whilst maintaining a low coercive field value, high saturation induction and excellent temperature stability.

### Example I

Nanocrystalline bulk rapidly-cooled alloy contains 65 % Fe atomically; B - 20 %; Zr - 2 %; Si - 0.25 %; Co - 10.75 %, Hf - 2 % and the inevitable impurities. In an example, they are 0.05 %.

Polycrystalline ingots, prepared earlier by established methods, are used to make batch quantities for the final melting. Plate-shaped nanocrystalline samples, of 0.5 mm thickness, are produced by a system that uses a method involving the injection of liquid alloy into a copper water-cooled mould. The entire casting process takes place within a vacuum chamber. The liquid alloy is injected into the copper mould from a quartz crucible. The actual form used was hollowed-out, to meet requirements for a future product.

The physical properties of the plate-shaped samples of this alloy, for the example production alloys, are as follows: wherein the Fe₆₅Co₁₁B₂₀Zr₂Hf₂ alloy is the template alloy:

| | **Alloy** | **Hc [A/m]** | **Ms [T]** | **D_{spf} [meV/nm²]** | **T_{C}[K]** |
|---|---|---|---|---|---|
| Template | Fe₆₅Co₁₁B₂₀Zr₂Hf₂ | 310 | 1.43 | 46 | 690 672 668 |
| Example I | Fe₆₅Co_{10.75}B₂₀Si_{0.25}Zr₂Hf₂ | 143 | 1.40 | 45 | |
| Example II | Fe₆₅Co_{10.5}B₂₀Si_{0.5}Zr₂Hf₂ | 56 | 1.40 | 43 | |
| Example III | Fe₆₅Co_{10.25}B₂₀Si_{0.75}Zr₂Hf₂ | 62 | 1.38 | 43 | 663 |
| Example IV | Fe₆₅Co₁₀B₂₀Si₁Zr₂Hf₂ | 61 | 1.37 | 43 | 655 |

### Example II

Nanocrystalline bulk rapidly-cooled alloy contains atomically Fe - 65 %; B - 20 %; Zr - 2 %; Si - 0.5 %; Co - 10.5 %, Hf - 2 % with impurities of 0.01 %.

### Example III

Nanocrystalline bulk rapidly-cooled alloy contains atomically Fe - 65 %; B - 20 %; Zr - 2 %; Si - 0.75 %; Co - 10.25 %, Hf - 2 % with impurities of 0.09 %.

### Example IV

Nanocrystalline bulk rapidly-cooled alloy contains atomically Fe - 65 %; B - 20 %; Zr - 2 %; Si - 1 %; Co - 10 %, Hf - 2 % with impurities of 0.07 %.

## Claims

1. Nanocrystalline bulk iron alloy, **characterised in that** it has the atomic composition Fe₆₅Co₁₁₋ₓB₂₀SiₓZr₂Hf₂, where the value of x is equal to: 0.25 or 0.5 or 0.75 or 1, and in which the permissible quantity of impurities does not exceed 0.09 %.
